

E. GAYFORD & G. CRERAR.  
PROCESS OF CONCENTRATING ORES.  
APPLICATION FILED MAY 29, 1914.

1,176,441.

Patented Mar. 21, 1916.



Inventors

Ernest Gayford.

George Crerar.

By T. Walter Fowler.

Attorney

Witnesses

M. J. Clegg  
G. Manning

# UNITED STATES PATENT OFFICE.

ERNEST GAYFORD AND GEORGE CRERAR, OF SALT LAKE CITY, UTAH, ASSIGNEES TO METALS RECOVERY COMPANY, OF AUGUSTA, MAINE, A CORPORATION OF MAINE.

## PROCESS OF CONCENTRATING ORES.

1,176,441.

Specification of Letters Patent. Patented Mar. 21, 1916.

Application filed May 29, 1914. Serial No. 841,710.

To all whom it may concern:

Be it known that we, ERNEST GAYFORD, a subject of the King of Great Britain, and GEORGE CRERAR, a citizen of the United States, residing at Salt Lake City, in the county of Salt Lake and State of Utah, have invented certain new and useful Improvements in Processes of Concentrating Ores, of which the following is a specification.

10 Our invention relates to a "buoyant" process for the concentration of metallic ores by separating the metallic particles from the barren or rocky constituents thereof, and the invention consists of the process

15 which we will hereinafter describe and claim.

Our process is specifically related to the art commonly known as "flotation processes" and which is distinct from the usual gravity 20 concentration processes, in which the particles are separated by their differences in weight, or specific gravity, in that in the flotation process a certain percentage of oil, or of two dissimilar oils, or an oil and an 25 acid, or an oil and an alkali, is mixed with finely ground ore pulp and the mixture is then subjected to a violent agitation with the result that large volumes of air are beaten into, impregnated or entrained by 30 the pulp for the purpose of producing a froth composed of bubbles of air and oil to which the mineral particles attach, said froth having the appearance of an aggregation or mass of fine soap bubbles which when 35 collected and the froth discharged or broken down, by natural settlement, by suction or vacuum, or by the addition of cold water, or other means, displaces the mineral particles that have been caught.

40 In the accompanying drawing we have illustrated diagrammatically, an apparatus capable of working our process and wherein the several parts of the apparatus are so arranged as to perform the process progressively or in a step-by-step manner.

45 In carrying out our process we first reduce the mineral-bearing material by some suitable mechanism and which may include an ore crusher, or a reducing mill, A, of any appropriate character, and in which mill the ore is reduced or crushed to a desired size, say such that it will pass through the meshes of a one-half inch screen, the crushing being, preferably, done with the ore in a dry condition. After being crushed or reduced to

the desired size, and an adequate amount of water and the necessary amount of oil, an oil and acid, or oil and an alkali, or material or substance having the property of producing a suitable froth with the ore is 60 mixed with the pulp and the mixture fed into a machine where it is wet ground or otherwise treated to further reduce the size of the particles. This second machine may, for instance, be represented by the well 65 known ball-mill, B, which will reduce the material so that it will pass a screen having meshes about 10 to the lineal inch, said mill having an inlet at one end to receive the material from the first grinding or reducing 70 machine and having an outlet at the opposite end for the discharge of the ground material therefrom. While we have shown and described a ball-mill as being suitable for the above purpose, it will be understood 75 that any standard machine capable of crushing or reducing the material may be substituted for the ball-mill without departing from the spirit of our invention.

Associated in proper relation with a discharge of the ball-mill or reducing machine, B, is a frothing flotation machine, C, of suitable character. A machine well adapted for this step of our process includes a tank having an inclined bottom provided with 80 one or more air cells, D, above which and forming the top of the same is a porous floor, E, through which air, gas, or vapor admitted under pressure into said cells will be discharged in a number of infinitely fine 85 streams into the body of pulp in the tank with the result that a froth, foam or suds is generated and which froth, foam or suds rises to the surface of the contents of the tank and is delivered through an overflow 90 lip or discharge, F, and finally is sent as a concentrate to a cleaning machine or bin. This frothing flotation machine, which we have illustrated in connection with our process forms no essential part of the present 95 invention and such specific machine is not specifically claimed by us, but is merely used for illustrative purposes, because it is found well adapted for our purpose and for the economical working out of our complete 100 process. In the frothing flotation machine, the heavier sands and coarser materials tend to settle upon the inclined porous floor, but because of the inclination of the said floor 105 they are caused to gravitate thereover to a 110

discharge, G. The machine, therefore, floats a concentrate and discharges a tailings in water. Succeeding the frothing flotation machine is another reducing machine, H, which may be of any suitable character, as a pebble-mill capable of reducing the material so that it will pass a screen of about 40 mesh per square inch. However, the character of this reducing machine is unimportant, provided it has the capacity to further reduce the ore, and the machine shown may be regarded as but representative of any mill or crushing apparatus suitable for the reduction of the tailings delivered from the preceding frothing flotation machine, C.

In introducing the tailings from the frothing flotation machine, C, into the aforesaid second reducing mill, H, for further reduction, we may also add to the tailings and its supply of water, a further amount of a suitable frothing agent, so that the further reduction of the ore, and which ore represents the tailings from the preceding frothing flotation machine, C, is done in the presence of a fresh supply of a suitable froth-producing agent, and there is thus the intimate admixture of this agent with the pulp during the further regrinding or further reduction of the material. Succeeding the second reduction mill, H, is another frothing flotation machine, I, of a character similar to the one before described, or of any other suitable character and in this machine a froth, foam or suds is produced in the manner similar to that before described, and the concentrates are caused to overflow or pass from this machine to the cleaning machine or bin or other depository. This machine, I, therefore, floats a concentrates and discharges a tailings in water, to which tailings a further amount of a suitable frothing agent, as before described, is added, if desired, and the tailings further reduced in size, if this is found to be desirable by re-crushing or further grinding in any standard machine, say a pebble-mill until the particles may pass a screen of say about 80 mesh. Thus, the material discharged from the reduction mill, H, is sent direct to a frothing flotation machine which in turn floats a concentrate, which is liberated by the recrushing, and discharges a tailings which in turn is reduced to a smaller size and sent to a frothing flotation machine and therein subjected to the action of the frothing agent, and the air, gas or vapor delivered into the same through the porous floor or bottom, as before described. These several operations are carried out until the point is reached when the recrushing and re-floating steps do not recover sufficient mineral to make them profitable, the final flotation machine discharging a tailings which has but little, if any, value.

From the foregoing, it will be understood

that our process involves crushing or reducing mineral-bearing material, by steps, to suitable sizes, and floating the liberated mineral at each crushing step, the number of the steps and the fineness of the crushing being 76 dependent upon the nature of the ore.

The results which we obtain from the practice of the foregoing process are superior to those which occur when the ore is crushed at once to the final size and then 75 treated by flotation, as it is a well known axiom in ore treatment, that the metal losses occur in the impalpable fine mineral made in crushing the ore and the finer the crushing the larger the amount of such impalpable 80 mineral, therefore, in our "step" flotation, the mineral liberated at each crushing is floated before the next step or before it is again subjected to a further and final reduction, which would reduce such mineral to an 85 undesirable condition were it not removed as soon as it is liberated from the gangue.

In all mineral-bearing material a portion of the mineral is liberated when the crushing is comparatively coarse, whereas 90 some is not liberated until the reduction is comparatively fine. We are aware that step crushing has been resorted to in ore dressing and we do not claim the same broadly as our invention, but step crushing 95 combined with step flotation has never been practised, as far as we know, and that portion of our process which involves the floating of the concentrates of each crushing step is novel and has resulted in the recovery 100 of a higher percentage of the mineral particles.

Apparatus such as we have described in the carrying out of our process is extremely simple and inexpensive. No mixing cells 105 are required, the mixture of the frothing agent and mineral being obtained in the crushing machine at each step; no complicated machinery is required, simply a crushing machine and a flotation machine for 110 each step.

Having thus described our invention what we claim as new and desire to secure by Letters Patent is:—

1. The process herein described, consisting, essentially, in progressively reducing, by successive stages, ore mixed with water and a frothable agent having a preferential affinity for metalliferous matter, aerating the mixture resulting from each reduction, and floating off the concentrates liberated at each reduction.

2. The process herein described which consists, essentially, in progressively reducing at intervals ore mixed with water and an oily agent having a preferential affinity for metalliferous matter, and aerating the mixture between successive reductions and floating off the concentrates liberated during a preceding reduction.

3. The process herein described which consists, essentially, in crushing ore mixed with water and a frothable agent having a preferential affinity for metalliferous matter, then aerating the mixture to buoy up and float off the concentrates liberated during the crushing, then further reducing the remaining tailings and aerating the mixture to buoy up and float off the concentrates liberated during the second reduction.

4. The ore concentrating process described herein which consists, essentially, in the step by step reduction of ore mixed

with water and a frothable agent having a preferential affinity for metalliferous matter, aerating the mixture following each step of the reduction and floating off the concentrates liberated at each reduction and previous to a succeeding reduction.

In testimony whereof we affix our signatures in presence of two witnesses.

ERNEST GAYFORD.  
GEORGE CRERAR.

Witnesses:

GEO. W. LUCAS,  
J. M. CALLOIS.